



- i) N, N'-bis(2-sulphoethyl)-dithio-oxamide, dipotassium salt  
 $\text{K}_2\text{O}_3\text{SCH}_2\text{CH}_2-\text{NH}-\text{C}(\text{S})-\text{C}(\text{S})-\text{NH}-\text{CH}_2\text{CH}_2\text{SO}_3\text{K}$
- ii) N, N'-bis(m-sulphobenzyl)-dithio-oxamide, diammmonium salt  

- iii) N-p-sulphophenyl-dithio-oxamide, sodium salt  

- iv) N, N'-diphenyl-dithio-oxamide  

- v) Bis-(dimethyl-thiocarbamoyl)-sulphide  

- vi) Bis-(piperidino-thiocarbonyl)-sulphide  


The optimum amounts to be applied of sulphur sensitizers according to the above general formula depend upon the compound chosen, the nature of the silver halide, the grain size, the desired ripening time, the ripening temperature, the pH and pAg of the silver halide emulsion. However, the amounts used generally vary from about 1 mg. to about 200 mg. per mole of silver halide. It is evident that smaller amounts of these compounds may be used too, e.g., when a little increase in sensitivity is envisaged. When using larger amounts care should be taken that no fog arises.

The new compounds may be used in combination with existing sensitizers such as tin (II) salts or thiourea dioxide. Very interesting additive increases in sensitivity are obtained when the new sensitizers are applied in combination with gold salts, such as gold thiocyanate, platinum salts and palladium salts. A considerable increase in sensitivity can also be obtained when applying the compounds according to the present invention in combination with development accelerators such as polyoxyalkylene derivatives having a molecular weight higher than 500 and onium compounds.

The new sulphur sensitizers can be used in spectrally as well as in not spectrally sensitized emulsions. They are successfully applied in common emulsions, in colour emulsions, in X-ray emulsions, in graphic emulsions, in Iippman emulsions and in fine grain emulsions for scientific purposes.

The classical emulsion ingredients such as stabilizers, antifogging agents, developing agents, hardening agents, colour couplers, softening agents, dispersing agents, etc., may be incorporated into the emulsion together with the sulphur sensitizers according to the invention without any detrimental interaction taking place.

Although the use of the sulphur sensitizers according to the above general formula is of great technological importance to sensitize silver halide emulsions prepared with inert gelatin, it is also very interesting to use them for the sensitization of silver halide emulsions the protective colloid of which at least partially consists of active ester or other hydrophilic colloids such as polyvinyl alcohol.

When necessary, the compounds may also be used in combination with known sulphur sensitizers in order to obtain special effects such as very high maximum densities and high gradations together with high sensitivities.

The following examples illustrate the present invention.

#### EXAMPLE 1

A silver bromo-iodide emulsion (3 mole percent of iodide) prepared with inert gelatin and having an average grain size of 0.5 micron, a pAg of 7.5 and a pH of 6.5 is divided into three equal parts (samples A, B and C). The sulphur sensitizers listed in Table I are added to samples B and C in the given concentrations. The emulsions are then ripened at 45° C. for 3 hours whereupon they are coated on a cellulose triacetate support. The test-strips obtained are developed after exposure in a hydroquinone-p-monomethyl-aminophenol hemisulphate developer, fixed and rinsed whereupon the speed is measured. In Table I the relative speeds are listed.

TABLE I

|    | Sulphur sensitizer | Concentration per mole of silver halide | Rel. speed |
|----|--------------------|-----------------------------------------|------------|
| 20 | A                  |                                         | 100        |
|    | B                  | $1.5 \times 10^{-5}$ mole               | 300        |
|    | C                  | $1.5 \times 10^{-6}$ mole               | 300        |

#### EXAMPLE 2

25 A gold thiocyanate solution is added in an amount equivalent to 5 mg. of gold per mole of silver halide to a same emulsion as described in Example 1 just before dividing the emulsion in samples A, B and C and before the addition of compounds 2 and 3 in the given concentration to samples B and C. The three samples are coated and further treated as described in Example 1. The materials according to the present invention show a sensitivity that is 3 times as high as that of the light-sensitive material containing only gold rhodanide and no chemical sensitizer according to the present invention.

#### EXAMPLE 3

An all-silver iodide emulsion prepared with inert gelatin and having a pAg of 9 and a pH of 6.5 is divided into 40 four equal parts A, B, C and D. To each part is added the chemical sensitizer listed in Table II hereinafter in the concentration given. After having been ripened for 1 hour at 50° C. the four emulsions are coated on a cellulose triacetate support. The light-sensitive materials obtained are exposed and further treated as described in Example 1. The relative speeds are given in Table II.

TABLE II

|    | Sulphur sensitizer | Concentration per mole of silver halide | Rel. speed |
|----|--------------------|-----------------------------------------|------------|
| 50 | A                  |                                         | 100        |
|    | B                  | Sodium thiosulphate $1.10^{-4}$ mole    | 100        |
|    | C                  | Compound 1 $1.10^{-4}$ mole             | 200        |
|    | D                  | Compound 5 $1.10^{-4}$ mole             | 150        |

#### EXAMPLE 4

An all-silver chloride emulsion prepared with inert gelatin and having an average grain size of 0.12 micron, a pAg of 7.5 and a pH of 6.5 is divided into three equal parts A, B and C. The compounds listed in Table III are added to each emulsion part in the concentration given. After an optimum ripening period of 1½ hours at 50° C. the three emulsions are coated on a cellulose triacetate support whereupon the materials obtained are further treated as described in Example 1. The relative speeds of the materials are listed in Table III.

TABLE III

|    | Sulphur sensitizer | Concentration per mole of silver halide       | Rel. speed |
|----|--------------------|-----------------------------------------------|------------|
| 70 | A                  |                                               | 100        |
|    | B                  | Sodium thiosulphate $0.7 \times 10^{-4}$ mole | 200        |
|    | C                  | Compound 10 $0.7 \times 10^{-4}$ mole         | 350        |

#### EXAMPLE 5

To the same kind of emulsion as described in Example 4 a gold thiocyanate solution is added, in an amount

equivalent to 7 mg. of gold per mole of silver halide, before dividing the emulsion into samples, and adding a chemical sensitizer according to the invention. The emulsion is divided into two equal parts and to one part  $0.7 \times 10^{-4}$  mole of compound 10 per mole of silver chloride is added. The emulsions are coated and further treated as described in Example 4. The speed of the light-sensitive material comprising compound 10 is 3 times as high as that of the other material.

## EXAMPLE 6

An ammoniacal silver bromo iodide emulsion (3 mole percent of iodide) which has been prepared with inert gelatin, and which has not been washed as was the case with the emulsions of the preceding examples, is divided immediately after its preparation into 3 equal parts (samples A, B and C). The sulphur sensitizers listed in Table IV are added to samples B and C in the given concentrations. After having been kept for 30 min. at 35° C. the three samples are coated onto a cellulose triacetate support and further treated as in Example 1. The relative speeds of the three materials are listed in Table IV.

TABLE IV

| Sulphur sensitizer         | Concentration per mole of silver halide | Rel. speed |
|----------------------------|-----------------------------------------|------------|
| A-----                     | -----                                   | 100        |
| B----- Sodium thiosulphate | $5 \times 10^{-5}$ mole-----            | 100        |
| C----- Compound 2-----     | $5 \times 10^{-5}$ mole-----            | 150        |

## EXAMPLE 7

240 cc. of a 3M aqueous silver nitrate solution and 240 cc. of a 3M aqueous potassium bromide solution are simultaneously and slowly added at 35° C. to a solution of 50 g. of gelatin in 500 cc. of water (emulsion A). A second emulsion is prepared in the same way with the only difference that the aqueous gelatin solution to which the aqueous silver nitrate and the potassium bromide solutions are added also comprises 9 mg. of compound 2 (emulsion B).

Emulsions A and B are physically ripened by keeping them for 60 min. at 45° C.

Electron micrographs (magnification 10,000  $\times$ ) are taken from the ripened liquid emulsions. In both cases, these micrographs show a dispersion of silver bromide grains ranging for the greater part from about 0.05 to about 0.1 $\mu$ . Emulsion A, however, also contains a considerable number of grains ranging from about 0.5 to about 1.0 $\mu$  whereas emulsion B only contains some grains which are of larger size than 0.1 $\mu$ . From the results obtained it clearly appears that the presence of a chemical sensitizer according to the present invention during the precipitation of the silver halide and the physical ripening of the emulsion obtained prevents in a very efficient way the formation of large silver halide grains.

We claim:

1. Photographic light-sensitive silver halide emulsion

containing as a sensitizer at least one compound corresponding to the following general formula:



wherein:

A is a sulphur atom,  
each of  $\text{R}_1$ ,  $\text{R}_2$ ,  $\text{R}_3$  and  $\text{R}_4$  is hydrogen, alkyl, or aryl, or  
 $\text{R}_1$  and  $\text{R}_2$  and/or  $\text{R}_3$  and  $\text{R}_4$  together are the atoms necessary to close a heterocyclic ring, and  
 $n$  is zero or one.

2. Photographic light-sensitive emulsion according to claim 1, wherein the silver halide emulsion includes a protective colloid consisting substantially of inert gelatin.

3. Photographic light-sensitive emulsion according to claim 1, wherein the emulsion is an unwashed silver halide emulsion.

4. Photographic light-sensitive emulsion according to claim 1, wherein the silver halide of the emulsion consists substantially of silver chloride.

5. Photographic light-sensitive emulsion according to claim 1, wherein the silver halide of the emulsion consists substantially of silver iodide.

6. Photographic material comprising a light-sensitive silver halide emulsion layer applied from the silver halide emulsion of claim 1.

7. The photographic light-sensitive emulsion of claim 1 wherein the emulsion is a fine grain emulsion.

8. Photographic light-sensitive emulsion according to claim 1, wherein the emulsion includes a polyoxyalkylene derivative having a molecular weight higher than 500.

9. Photographic light-sensitive emulsion according to claim 1, wherein the emulsion includes an onium compound.

10. Photographic light-sensitive emulsion according to claim 1, wherein the sensitizer is present in an amount of from 1 to 200 mg. per mole of silver halide.

11. Photographic light-sensitive emulsion according to claim 1, wherein the emulsion includes a gold salt.

12. Photographic light-sensitive emulsion according to claim 11, wherein said gold salt is gold thiocyanate.

## References Cited

## UNITED STATES PATENTS

3,226,232 12/1965 Dersch et al. ----- 96—107 X  
3,287,137 11/1966 McBride ----- 96—107

50 NORMAN G. TORCHIN, Primary Examiner

A. T. SUROPICO, Assistant Examiner

U.S. CL. X.R.

96—108